

## UNITED STATES PATENT OFFICE.

ARCHIBALD JOHN HALL, OF TIMBERSBROOK, CONGLETON, ENGLAND, ASSIGNOR TO  
CELANESE CORPORATION OF AMERICA, A CORPORATION OF DELAWARE.

## TREATMENT OF CELLULOSE ACETATE ARTIFICIAL SILK.

No Drawing. Application filed June 8, 1928, Serial No. 283,998, and in Great Britain June 8, 1926.

This invention relates to processes for the treatment of cellulose acetate artificial silk so that it acquires permanent resistance to deterioration during treatment with hot or 5 boiling aqueous media.

It is well known that cellulose acetate artificial silk, unlike the artificial silks of the regenerated cellulose type i. e. viscose, cuprammonium and the so-called nitrocellulose artificial silks, when subjected to the action of moist steam, boiling water or water at a temperature exceeding about 90° C. becomes curly and wool-like and suffers a considerable loss of lustre. Consequently in the treat-

15 15 treatment of yarns, fabrics and other materials containing cellulose acetate artificial silk, steaming treatments and treatments with aqueous liquors of a temperature exceeding about 80° C. have to be avoided. This fact

20 20 is somewhat disadvantageous to the use of cellulose acetate artificial silk as compared with the regenerated cellulose artificial silks, which, as indicated above, are not in general subject to such deterioration.

25 25 According to the present invention cellulose acetate artificial silk in whatever form, provided it is in the set condition, is stretched beyond its elastic limit, whereby it is rendered much more resistant to deterioration on

30 30 treatment with hot aqueous media and may even retain its original lustre and not become curly and wool-like when immersed in boiling water for prolonged periods. The effect of the stretching is entirely new technically,

35 35 no process being known which renders cellulose acetate artificial silk permanently more resistant to treatment with hot aqueous media.

40 40 It is essential that the cellulose acetate artificial silk should be in the set condition before being subjected to the stretching operation. In fact, if the artificial silk is not set the operation would amount to little more than the stretching which is customarily applied in the production of the artificial silk filaments (the so-called "stretch-spinning" process), and as is well known the filaments so produced under stretch are liable to the above described deterioration.

45 45 In carrying out this invention, cellulose acetate artificial silk at any stage in its production after the silk is in the set condition is stretched beyond its elastic limit in a dry or wet condition for the purpose of preserving its lustre and appearance. The stretching

process may be carried out after treatment with one or more softening or swelling agents for the cellulose acetate. Such softening or swelling agents (hereinafter referred to collectively as swelling agents), may be employed in any suitable manner, for example dissolved in aqueous or organic solvents, or in the form of vapour, and the silk may be subjected to their action for any suitable period of time or at any suitable temperature. 60 Generally it is preferred to stretch the silk before removal of the swelling agent or agents although in certain instances it may be desirable to remove the swelling agent before or during stretching. After stretching, 65 the swelling agent may be removed from the yarn by washing with water or otherwise and the silk may then be dried in any suitable manner.

70 70 Examples of suitable swelling agents are acetone, ethyl alcohol, formaldehyde and glycerine.

75 75 The effect of stretching on the lustre and appearance of cellulose acetate silk is largely determined by the degree of stretching. Generally, it is found that the greater the stretching the greater the resistance of the resulting yarn to deterioration when immersed in boiling water. For instance, cellulose acetate silk yarn of 3000 to 4000 denier, wetted with 80 water and stretched 10% in length, and afterwards immersed for 15 minutes in boiling water becomes slightly curly or wool-like and somewhat less lustrous. On the other hand, similar yarn treated for one hour at 15-20° 85 C. with a 20% aqueous solution of acetone and afterwards stretched 25% in length, does not become wool-like and retains practically the whole of its lustre when immersed for one hour in boiling water. 90

95 95 Accordingly, it is preferred in carrying out this invention to treat the cellulose acetate silk with a swelling agent before stretching, since this treatment causes the cellulose acetate to swell and allows the maximum stretching to be obtained without breakage or substantial breakage of the silk filaments. 100

This invention is not limited to the use of any special swelling agent or any limits of stretching beyond the elastic limit but consists essentially in stretching cellulose acetate silk filaments after the silk is in the fully set and finished condition so that they have the desired resistance to deterioration in hot or boiling aqueous solution, the filaments be- 105 110

ing preferably treated before stretching with any swelling agent for cellulose acetate.

It is to be understood that the invention may be applied to cellulose acetate silk whether in the form of skeins, or single yarns, and when present in any manufactured fabric.

It is found that stretching of 15-25% in length yields satisfactory resistance to hot or boiling aqueous liquors with cellulose acetate silk yarn of 3000 to 4000 denier.

Cellulose acetate yarns of relatively high denier may be stretched to produce yarns of lower denier and if stretched sufficiently the resulting finer yarns will be wholly or partially resistant to deterioration when subsequently immersed in hot or boiling aqueous solutions. The yarns may be treated before stretching with suitable swelling agents.

The following examples indicate methods for carrying out this invention although it must be clearly understood that it is not limited in any way to the conditions described therein.

*Example 1.*

Cellulose acetate silk yarn of 3000-4000 denier is stretched 15% in length. The resulting yarn has good resistance to boiling water.

*Example 2.*

Cellulose acetate yarn of about 300 denier is steeped in a 15% aqueous solution of acetone for one hour at 16° C., then stretched 15% in length, washed in water for complete removal of acetone and dried. The resulting yarn withstands boiling water for at least one hour.

*Example 3.*

Cellulose acetate silk yarn of about 3000 denier is steeped for 1/2 hour at 20° C. in 20% aqueous solution of ethyl alcohol, then stretched 25%, washed in water and dried. The resulting yarn has excellent resistance to boiling water for at least one hour.

What I claim and desire to secure by Letters Patent is:—

1. Process for the treatment of cellulose acetate artificial silk, comprising stretching the artificial silk in the set condition beyond its elastic limit, whereby it is rendered more resistant to deterioration by hot aqueous media.

2. Process for the treatment of cellulose

acetate artificial silk, comprising treating the artificial silk in the set condition with a swelling agent for cellulose acetate and then stretching it beyond its elastic limit, whereby it is rendered more resistant to deterioration by hot aqueous media. 55

3. Process for the treatment of cellulose acetate artificial silk, comprising treating the artificial silk in the set condition with a swelling agent for cellulose acetate and then stretching it beyond its elastic limit and removing the swelling agent, whereby the 65 artificial silk is rendered more resistant to deterioration by hot aqueous media.

4. Process for the treatment of cellulose acetate artificial silk, comprising treating the artificial silk in the set condition with a swelling agent for cellulose acetate at ordinary 70 temperature and then stretching it beyond its elastic limit, whereby it is rendered more resistant to deterioration by hot aqueous media.

5. Process for the treatment of cellulose acetate artificial silk, comprising treating the artificial silk in the set condition with a swelling agent for cellulose acetate and then stretching it by 15-25% of its length, whereby it is rendered more resistant to deterioration 80 by hot aqueous media. 75

6. Process for the treatment of cellulose acetate artificial silk, comprising treating the artificial silk in the set condition with a swelling agent for cellulose acetate and then stretching it by 15-25% of its length and removing the swelling agent, whereby the 85 artificial silk is rendered more resistant to deterioration by hot aqueous media.

7. Process for the treatment of cellulose acetate artificial silk, comprising treating the artificial silk in the set condition with an aqueous solution of acetone and then stretching it beyond its elastic limit, whereby it is rendered more resistant to deterioration by 95 hot aqueous media. 90

8. Process for the treatment of cellulose acetate artificial silk, comprising treating the artificial silk in the set condition with an aqueous solution of acetone and then stretching it by 15-25% of its length, whereby it is rendered more resistant to deterioration by 100 hot aqueous media.

In testimony whereof, I have hereunto subscribed my name.

ARCHIBALD JOHN HALL.